

F. D. CARNEY & L. B. LINDEMUTH.  
METHOD OF MAKING SOUND CASTINGS.  
APPLICATION FILED JUNE 12, 1913.

1,073,735.

Patented Sept. 23, 1913.



Witnesses

B. Wommers  
C. Leckert.

Inventors

Frank D. Carney  
Lewis B. Lindemuth  
Henry Orth Jr. Attorney

# UNITED STATES PATENT OFFICE.

FRANK D. CARNEY AND LEWIS B. LINDEMUTH, OF STEELTON, PENNSYLVANIA.

## METHOD OF MAKING SOUND CASTINGS.

1,073,735.

Specification of Letters Patent. Patented Sept. 23, 1913.

Application filed June 12, 1913. Serial No. 778,291.

To all whom it may concern:

Be it known that we, FRANK D. CARNEY and LEWIS B. LINDEMUTH, both citizens of the United States of America, and residents of Steelton, Dauphin county, Pennsylvania, have invented certain new and useful Improvements in Methods of Making Sound Castings; and we do hereby declare the following to be a full, clear, and exact description of the invention, such as will enable others skilled in the art to which it appertains to make and use the same, reference being had to the accompanying drawings, and to letters or figures of reference marked thereon, which form a part of this specification.

This invention relates to the method of making sound castings, and more especially to the making of sound castings containing large volumes of metal, such as ingots and the like, the object being to reduce or eliminate the pipe, and reduce the quantity of metal in the "crop" ends, thereby saving much valuable metal from being "scrapped."

Hereinafter we shall refer to the ingot, as a type of casting containing a large volume of metal, but wish it understood that the operations hereinafter described are equally applicable to other shapes and types of large castings.

In casting an ingot, for example, the metal is poured or teemed in the usual manner into the ingot mold. After the desired quantity of metal has been placed in the mold the top surface is blanketed with an insulating layer of any suitable material, such as a slag, preferably a low fusing slag having good insulating properties; or it may be blanketed by adding materials capable of forming such a slag when said materials are heated by the molten metal in the mold without injuriously chilling the metal, or by adding a fuel, as charcoal or coke, as the insulating material. An open-ended form is then placed or floated on the molten metal, preferably a frustum whose major diameter is considerably less than the diameter of the top of the ingot mold. This form may be floated on the metal either before or after placing the blanket thereon. The most practical form is the frustum of a cone or of a square pyramid. The base of the frustum is preferably formed with a large bearing surface, either by thickening the lower end, or by forming an external flange on said end. Any material fusing at a high

temperature may be used, fire-clay having been found quite suitable. Care should be taken that the frustums are thoroughly dry, to prevent explosions and injury to the workmen, and if desired, they may be heated to any desired temperature before being placed on the molten metal in the mold. As the metal sets the frustum becomes fastened in the metal, or, as it were, "frozen" in place. It is necessary for the subsequent operations, that the form be held, as otherwise it would rise when additional molten metal is added. When the metal has set, or even before this has taken place, it is preferable, but not necessary to place additional insulating material on top of the blanket in the annular space between the frustum and the inner walls of the mold to a depth approximately the height to which the frustum projects above the metal surface in the mold, that is to say, about on a level with the top of the frustum. After about one-third to one-half the total volume of the ingot has set or solidified, a depression forms in the molten center of the ingot, which is about one-half the volume of the pipe, were such allowed to be formed. Molten metal is then poured through the frustum into the depression until the frustum is filled or about filled with this added metal.

It is well understood in present practice that molten iron or steel when in condition for casting is of a much lower temperature than the highest temperature of the furnace, the aim being to have the metal at as low a temperature as possible and still sufficiently limpid or fluid to fulfil all the conditions for casting, and also with the aim to produce a casting with as little "pipe" as possible. It is also well known that segregation takes place at the center of the ingot to a greater or less extent, according to the composition of the metal and its rate of cooling. Now, according to our process, the added molten metal above referred to, may be of the same composition as the metal cast in the mold, or it may be of a different composition. When the added molten metal is of a different composition, such composition is chosen as will reduce the average of the segregated elements to that average these elements have in the already set portion of the ingot, the aim being to produce an ingot having a uniform composition throughout.

When the added molten metal is of the same composition as that first placed in the

- mold, segregation is broken up and distributed over a large volume by the stirring action of the molten stream of metal striking that fluid portion of the ingot in which the 5 segregation had already commenced. By thus distributing the segregation over a large volume the degree of segregation in any one place is so reduced as to render it harmless in many cases. Of course, the degree or extent of the stirring action is dependent upon the extent of drop of the hot metal addition, in other words, upon the distance of the ladle or other device containing the molten addition above the form, and consequently the degree of mixing is to a great extent within the control of the person carrying out the invention. According to our 15 invention we also have this molten, and preferably purer, addition of high temperature, that is to say, the temperature of the molten metal added is higher than that of the greater volume of metal first placed in the mold. When this additional molten metal is poured or teemed into the form, it sinks 20 through the blanket of slag or other material that is inside the form, and first fills the depression above mentioned, and then rises in the form, at the same time raising the blanket on its surface. This raised portion of the 25 blanket on the hot molten metal addition in the form now prevents the added metal from cooling too rapidly. The segregated area within the ingot, which was still molten at the time the hot metal was added, now receives 30 heat from the hotter molten addition. The segregated volume contains a greater percentage of metalloids than the molten addition, and, being lighter, it rises and mixes with and diffuses in the purer metal (of the same, or different composition, as the body 35 of metal first poured) as above described. The center then cools down, (segregation and tendency to pipe still continuing, the segregated area being lifted wholly or partially into the body of metal added,) and this added metal sinks, to follow up the 40 shrinkage due to cooling, and effectually prevents the formation of a pipe in the ingot proper.
- 45 It will be noted that no mechanical means are used to hold the form in place, this being done by the molten metal itself, and that the form need not be of undue weight to hold it down, it being only sufficiently strong to withstand the hydrostatic pressure due to the height of the added metal above the level 50 of the upper surface of the ingot proper.
- The form being of much less diameter than the upper surface of the ingot enables it to be quickly inserted in the mold at the proper time, and also reduces the volume of metal to be scrapped.
- 55 Another, most important, advantage results from the use of this method of making sound castings, in that the ingot mold may

be filled to any depth desired, thereby avoiding the necessity of providing different sized molds for ingots of different weight, as it is immaterial to what depth the mold is filled when this form is used. Thus, ingots may 70 be cast in the same mold suitable for rolling rails of 60, 80 or 100 pounds to the yard, and with the same sized form.

It is immaterial what method is used in fixing or freezing the form in place. 75

When the metal, in casting condition, is found to be sufficiently hot when first poured or teemed into the mold to give plenty of time for the various manipulations, the form may at once be floated on its surface and frozen into place by causing a skin to form on the annular surface between the outer walls of the bottom of the frustum and the inner walls of the ingot mold; and this may be done by packing this annular space with 80 molder's sand, or the equivalent, the aim being to maintain the surface portion of the metal inside the form in such a condition that the molten addition may combine with the segregated area and follow up the 85 shrinkage, and form a solid ingot as homogeneous throughout as possible. 90

We are aware that it has heretofore been proposed to blanket an ingot top with the idea of reducing the volume of the pipes, but 95 practice demonstrates that the volume remains substantially the same, though the shape is considerably altered.

Our purpose in using a blanket is, primarily to prevent too rapid cooling, and preserve the top molten only for a sufficient length of time to permit the insertion of the form, and to maintain the surface of the casting within the form in proper condition until metal can be conveniently added to 105 produce the result we attain.

Referring to the accompanying drawings, in which like parts are similarly designated, Figures 1, 2 and 3 are vertical sections of an ingot mold intended to illustrate our process 110 at different stages; Fig. 4 is a similar view of the ingot. Figs. 5, 6 and 7 are views similar to Figs. 1, 2 and 3, but where the mold is not cast full. Figs. 8, 9 and 10 are modified forms of fire-clay forms. 115

The ingot mold 1 in Fig. 1, is indicated as containing molten metal at 2, with a molten slag covering 3 and a cylindrical form 4 floated thereon, the space between the mold 1 and form 4 being filled with molder's 120 sand 5.

In Fig. 2 the metal is supposed to have partially solidified, as indicated at 2<sup>a</sup> adjacent the sides of the mold 1, leaving a central molten portion 6, intended to indicate the area of segregation. It will be noted that the slag layer within the form 4 is thicker, indicating that additional slag or slag forming material has been placed in the form with carbonaceous material 7 on 130

top. The latter may be omitted if found unnecessary. The central depression is indicated at 8 filled with slag.

In Fig. 3 the added metal has been placed 5 in the form; the molten slag layer 3<sup>a</sup> within the form has floated on the top of the added metal, and the area of segregation 6<sup>a</sup> is shown as raised and smaller, extending into the form with the slag layer 3<sup>a</sup> on top.

10 In Fig. 4 we have shown the ingot removed from the mold and the form broken away, and showing a few recesses or holes 9 in the neck below the slag layer 3<sup>a</sup>.

Figs. 5, 6 and 7 are identical with Figs. 15 1, 2 and 3, except that there is less metal shown in the molds 1.

Figs. 8, 9 and 10 show different forms of frusta. In Fig. 8 the walls of the frustum 10 are of uniform thickness, while in Fig. 9 20 they are tapered, being thicker at the bottom of the frustum 11. In Fig. 12 the frustum 11 is shown as having an external base flange 12.

We claim—

25 1. The method of making sound castings, which comprises pouring molten metal into a mold to any desired depth, placing a form on the metal therein and allowing it to freeze in place, and then pouring into the 30 form, while the center of the casting is still molten, an additional quantity of metal.

2. The method of making sound castings, which comprises pouring molten metal into a mold to any desired depth, placing a form 35 on the metal therein and allowing it to freeze in place, and then pouring into the form, while the center of the casting is still molten, an additional quantity of metal of a composition calculated to mix with the 40 molten metal to form a composition substantially the same as that of the body of the casting.

3. The method of making sound castings, which comprises filling a mold to the desired 45 depth, freezing an open-ended form on the surface of the metal in the mold while maintaining the center of the casting molten and its surface metal within said 50 form in condition for the reception of a subsequent quantity of molten metal, then placing in the form such molten metal, said added metal being of a temperature higher than the temperature of the molten center of the casting.

55 4. The method of making sound castings, which comprises filling a mold to the depth desired, freezing an open-ended form in

the top of the metal, while the center of the casting is still molten, then filling said form with molten metal having a temperature 60 higher than that of the metal first placed in the mold.

5. The method of making sound castings, which comprises filling a mold to the depth desired, freezing an open-ended form in the top of the casting and pouring into said form hot molten metal, after one-third to one-half of the volume of the casting has solidified.

6. The method of making sound castings, 70 which comprises pouring molten metal into a mold to any desired depth, blanketing the metal, floating a form on the blanketed metal and permitting said form to freeze in place, and pouring hotter molten metal into 75 and through said form.

7. The method of making sound castings, which comprises filling a mold to the depth desired, placing an open-ended form in the top of the metal, blanketing the surface of 80 the metal within the form, freezing the form in position and placing hot metal in the form.

8. The method of making sound castings, which comprises filling a mold to the depth 85 desired, blanketing the top of the metal with slag, floating an open-ended form on the surface of the metal, said form being frozen in place, packing the annular space between the exterior surface of the form 90 and the interior surface of the mold with refractory packing material and filling the form with an additional quantity of hot metal poured or teemed through the slag layer within the hollow form. 95

9. The method of making sound castings, which comprises pouring molten metal into a mold to any desired depth, placing a form on the metal therein and allowing it to freeze in place, and then pouring into the 100 form, while the center of the casting is still molten, an additional quantity of metal, and controlling the degree of mixing of the metal added by regulating the distance the added metal drops before entering the form. 105

In testimony that we claim the foregoing as our invention, we have signed our names in presence of two subscribing witnesses.

FRANK D. CARNEY.  
LEWIS B. LINDEMUTH.

Witnesses:

GEO. W. PARSONS,  
CHAS. R. HOLTON.